

## UNITED STATES PATENT OFFICE.

MATTHEW BARRATT MOORE, OF COVENTRY, ENGLAND.

## COMPOSITION FOR POLISHING CELLULOID SURFACES.

No Drawing. Application filed June 18, 1925, Serial No. 38,103, and in Great Britain May 27, 1924.

This invention has for its object to provide a simple process for producing a high-class finish on celluloid or surfaces which have been coated with a celluloid solution, 5 celluloid varnish, or other suitable celluloid preparation.

According to this invention, the surface is rubbed down, and friction-polished, with a composition comprising a suitable solvent 10 of celluloid and a very fine cutting, levelling, and polishing grit, to which is added a lubricant, whereby the surface is levelled without appreciably adding to nor removing from the material forming the surface.

15 I prefer to employ either methylated spirits or turpentine, or both, in equal parts, as the solvent, and Vienna chalk for the fine cutting, levelling and polishing grit.

For the lubricant, paraffin oil, linseed or 20 other suitable oil, or both, may be used.

It is an essential feature of the invention that during the polishing process nothing is added to nor appreciably removed from the existing surface. Any roughness of the latter is eliminated by a levelling action which transfers the crests of such roughness into the depressions thereof so that they are filled and the surface is thereby made smooth.

25 In the preferred method of carrying out this invention, a composition is employed comprising equal parts in bulk of methylated spirits and turpentine, and a quarter of the bulk of that mixture in Vienna chalk, with a lubricant. These are mixed together 30 and applied to a rag, cotton wool, rubber, bob or the like, with which the surface is then polished. The polishing is carried out so as to rub down the surface and polish it, and therefore it is done comparatively 35 quickly and forcibly, as in ordinary polishing. This smoothens the surface, which dries rapidly.

40 In many cases the resultant finish is all that is desired, but, where a very high class finish is required, a further composition is used comprising four parts each by bulk of the solvent and of the fine cutting and polishing grit, and one part by bulk of linseed oil or paraffin. In making this composition, 45 preferably turpentine, methylated spirits, and linseed oil or paraffin oil, are mixed together. The Vienna chalk is made into a paste separately with methylated spirits to about the consistency of cream, and is then 50 added. The mixture is then applied to a rag, cotton wool, rubber, bob or the like, and

the surface well rubbed down and polished with it.

The final finish resembles either a high class varnished or polished surface. 60

It is understood that the proportions of the different materials given are not binding, and are only given as examples for producing a composition which will enable goods results to be obtained. The proportions may be varied, and the specific ingredients changed for others having equivalent effects, the essential feature being that the process involves friction polishing by the aid of a suitable solvent of the celluloid in conjunction with a fine cutting, levelling, and polishing grit. Generally, the solvent must be of a mild nature such as those specified, acetone being, in most cases, too active. 75

The process can be used for celluloid coatings on wood of coarse grain, provided that the grain has been sufficiently filled before being sprayed with celluloid. It can also be used for celluloid coating upon metal, and 80 the metal may have been tinted or coloured before being coated with celluloid and before the subsequent polishing process. In some circumstances it can also be used upon celluloid sheets. It can also be used on surfaces coated with coloured celluloid preparations, such as celluloid paints or enamels. 85

It is essential to add some linseed oil or paraffin to the composition to act as a lubricant and reduce the effect of the solvent on the surface. 90

An additional advantage arising out of the invention is that a surface once polished by this process can, when scratched or damaged, have its surface made good by a further 95 polishing process embodying the celluloid solvent and fine grit, with a lubricant.

What I claim as my invention and desire to secure by Letters Patent of the United States is:—

100 1. A composition for polishing celluloid surfaces consisting of four parts of a celluloid solvent, four parts of grit, and one part of lubricant, all by volume.

105 2. A composition for polishing celluloid surfaces consisting of two parts of methylated spirits, two parts of spirits of turpentine, four parts of Vienna chalk, and one part linseed oil, all by volume.

110 In testimony whereof I have signed my name to this specification.

MATTHEW BARRATT MOORE.